

# United States Patent [19]

McCrossen et al.

[11] 3,779,765

[45] Dec. 18, 1973

[54] **SILVER HALIDE EMULSIONS  
CONTAINING COUPLER SOLVENTS**

[75] Inventors: **Fred C. McCrossen; Harland J. Osborn**, both of Rochester, N.Y.

[73] Assignee: **Eastman Kodak Company**, Rochester, N.Y.

[22] Filed: **Aug. 31, 1972**

[21] Appl. No.: **285,288**

[52] U.S. Cl. .... **96/56.5, 96/55, 96/56,  
96/74, 96/100**

[51] Int. Cl. .... **G03c 7/00, G03c 1/40**

[58] Field of Search ..... **96/56.5, 55, 100**

[56] **References Cited**

UNITED STATES PATENTS

3,287,134 11/1966 Kainrath et al. .... **96/100**

|           |         |                     |               |
|-----------|---------|---------------------|---------------|
| 3,409,439 | 11/1968 | Yoshida et al. .... | <b>96/100</b> |
| 3,413,123 | 11/1968 | Nittel et al. ....  | <b>96/100</b> |
| 3,554,755 | 1/1971  | Rinauro ....        | <b>96/100</b> |
| 3,676,141 | 7/1972  | Hara et al. ....    | <b>96/100</b> |

Primary Examiner—J. Travis Brown  
Attorney—Robert W. Hampton et al.

[57]

## ABSTRACT

A method of obtaining color records of improved heat stability, also novel photographic emulsions and elements characterized by using one or more aliphatic or trimellitic- or trimethyl 1,3 pentane-diol diesters, or corresponding polyesters, as permanent coupler solvents.

**29 Claims, No Drawings**

# SILVER HALIDE EMULSIONS CONTAINING COUPLER SOLVENTS

This invention relates to color photography and particularly to improved color photographic elements and a method for efficiently incorporating substantially non-diffusible color couplers into one or more silver halide emulsion layers or a color photographic element to obtain photographic dyes of improved stability.

Color photographic elements containing hydrophobic dye-forming couplers dispersed in one or more light sensitive emulsion layers are well known in the art. Generally speaking, such elements contain a support and a plurality of sensitized silver halide gelatin emulsion layers such as red-, green- and blue-sensitive emulsions applied thereto; each of said emulsion layers, in turn, normally contain dispersed particles consisting of one or more dye-forming couplers wholly or partly dissolved in a permanent high boiling coupler solvent or encapsulated in a polymeric or wax-like material (ref. French Patents 2,017,718, 1,555,663 and U.S. Pat. No. 2,772,163).

In preparing such coupler-containing silver halide emulsions, it is customary to dissolve the coupler in a

activity with oxidized developing agents, there is a continuing need for more efficient solvent systems and techniques for utilizing couplers in general color photographic systems.

It is an object of the present invention to improve the efficiency and stability of coupler dispersions within photographic silver halide emulsions and also to improve the heat stability of the photographic record obtained when the dispersed couplers are reacted with oxidized color developing agents and processed.

These and other objects are obtained by utilizing in the usual manner as permanent coupler solvent one or more esters of the group:



high boiling coupler solvent such as tricresyl phosphate, then mill the coupler solution into an aqueous gelatin solution with a surfactant and, thereafter, combine the resulting dispersion with a light-sensitive gelatino-silver halide emulsion. For such purpose, the ratio of coupler-to-solvent can usefully vary from about 0.5-1.2-3 (ref. Jelley U.S. Pat. Nos. 2,322,027 and 2,801,171). The true solubility of most color-forming couplers, however, is considerably lower than suggested by the above ratio. In some cases, the solubility of the coupler is in the area of about one part coupler-to-ten parts of coupler solvent. As a result, the dispersed droplets of coupler solution in the emulsion layer are supersaturated. Despite this fact, the presence of even a minimal amount of coupler solvent is considered a disadvantage for general color photographic purposes. Emulsion layers thickened by coupler solvents tend to be less durable and image resolution of poorer quality. For this reason, continuing efforts are being made to cut down on the amount of solvent without corresponding loss in coupler reactivity or dye stability. For example, known high boiling crystalloidal coupler solvents have been used in combination with removable "auxiliary" solvents to initially dissolve the coupler (ref. Julian U.S. Pat. No. 2,949,360; Mannes U.S. Pat. No. 2,304,939; Jelley et al. U.S. Pat. No. 2,322,827; Vittum U.S. Pat. No. 2,801,170; Fierke U.S. Pat. Nos. 2,801,171 and 2,490,749; Rinaura U.S. Pat. No. 3,554,755, Thirtle et al. U.S. Pat. No. 2,835,579; Sawdey U.S. Pat. No. 2,533,514). Improved photographic emulsions of interest are generally summarized, for instance, in Section XXII, page 110, lines 1-50 of Product Licensing Index, Vol. 92, Publication 9232 (Dec., 1971).

Because of a marked difference in solubility among the best known couplers, and variations in coupler re-

45 (F)

50 55 60 65 66 67 68 69 70 71 72 73 74 75 76 77 78 79 80 81 82 83 84 85 86 87 88 89 90 91 92 93 94 95 96 97 98 99 100 101 102 103 104 105 106 107 108 109 110 111 112 113 114 115 116 117 118 119 120 121 122 123 124 125 126 127 128 129 130 131 132 133 134 135 136 137 138 139 140 141 142 143 144 145 146 147 148 149 150 151 152 153 154 155 156 157 158 159 160 161 162 163 164 165 166 167 168 169 170 171 172 173 174 175 176 177 178 179 180 181 182 183 184 185 186 187 188 189 190 191 192 193 194 195 196 197 198 199 200 201 202 203 204 205 206 207 208 209 210 211 212 213 214 215 216 217 218 219 220 221 222 223 224 225 226 227 228 229 230 231 232 233 234 235 236 237 238 239 240 241 242 243 244 245 246 247 248 249 250 251 252 253 254 255 256 257 258 259 260 261 262 263 264 265 266 267 268 269 270 271 272 273 274 275 276 277 278 279 280 281 282 283 284 285 286 287 288 289 290 291 292 293 294 295 296 297 298 299 300 301 302 303 304 305 306 307 308 309 310 311 312 313 314 315 316 317 318 319 320 321 322 323 324 325 326 327 328 329 330 331 332 333 334 335 336 337 338 339 340 341 342 343 344 345 346 347 348 349 350 351 352 353 354 355 356 357 358 359 360 361 362 363 364 365 366 367 368 369 370 371 372 373 374 375 376 377 378 379 380 381 382 383 384 385 386 387 388 389 390 391 392 393 394 395 396 397 398 399 400 401 402 403 404 405 406 407 408 409 410 411 412 413 414 415 416 417 418 419 420 421 422 423 424 425 426 427 428 429 430 431 432 433 434 435 436 437 438 439 440 441 442 443 444 445 446 447 448 449 450 451 452 453 454 455 456 457 458 459 460 461 462 463 464 465 466 467 468 469 470 471 472 473 474 475 476 477 478 479 480 481 482 483 484 485 486 487 488 489 490 491 492 493 494 495 496 497 498 499 500 501 502 503 504 505 506 507 508 509 510 511 512 513 514 515 516 517 518 519 520 521 522 523 524 525 526 527 528 529 530 531 532 533 534 535 536 537 538 539 540 541 542 543 544 545 546 547 548 549 550 551 552 553 554 555 556 557 558 559 560 561 562 563 564 565 566 567 568 569 570 571 572 573 574 575 576 577 578 579 580 581 582 583 584 585 586 587 588 589 5810 5811 5812 5813 5814 5815 5816 5817 5818 5819 5820 5821 5822 5823 5824 5825 5826 5827 5828 5829 5830 5831 5832 5833 5834 5835 5836 5837 5838 5839 5840 5841 5842 5843 5844 5845 5846 5847 5848 5849 5850 5851 5852 5853 5854 5855 5856 5857 5858 5859 5860 5861 5862 5863 5864 5865 5866 5867 5868 5869 58610 58611 58612 58613 58614 58615 58616 58617 58618 58619 58620 58621 58622 58623 58624 58625 58626 58627 58628 58629 58630 58631 58632 58633 58634 58635 58636 58637 58638 58639 58640 58641 58642 58643 58644 58645 58646 58647 58648 58649 58650 58651 58652 58653 58654 58655 58656 58657 58658 58659 58660 58661 58662 58663 58664 58665 58666 58667 58668 58669 58670 58671 58672 58673 58674 58675 58676 58677 58678 58679 58680 58681 58682 58683 58684 58685 58686 58687 58688 58689 58690 58691 58692 58693 58694 58695 58696 58697 58698 58699 586100 586101 586102 586103 586104 586105 586106 586107 586108 586109 586110 586111 586112 586113 586114 586115 586116 586117 586118 586119 586120 586121 586122 586123 586124 586125 586126 586127 586128 586129 586130 586131 586132 586133 586134 586135 586136 586137 586138 586139 586140 586141 586142 586143 586144 586145 586146 586147 586148 586149 586150 586151 586152 586153 586154 586155 586156 586157 586158 586159 586160 586161 586162 586163 586164 586165 586166 586167 586168 586169 586170 586171 586172 586173 586174 586175 586176 586177 586178 586179 586180 586181 586182 586183 586184 586185 586186 586187 586188 586189 586190 586191 586192 586193 586194 586195 586196 586197 586198 586199 586200 586201 586202 586203 586204 586205 586206 586207 586208 586209 586210 586211 586212 586213 586214 586215 586216 586217 586218 586219 586220 586221 586222 586223 586224 586225 586226 586227 586228 586229 586230 586231 586232 586233 586234 586235 586236 586237 586238 586239 586240 586241 586242 586243 586244 586245 586246 586247 586248 586249 586250 586251 586252 586253 586254 586255 586256 586257 586258 586259 586260 586261 586262 586263 586264 586265 586266 586267 586268 586269 586270 586271 586272 586273 586274 586275 586276 586277 586278 586279 586280 586281 586282 586283 586284 586285 586286 586287 586288 586289 586290 586291 586292 586293 586294 586295 586296 586297 586298 586299 586300 586301 586302 586303 586304 586305 586306 586307 586308 586309 586310 586311 586312 586313 586314 586315 586316 586317 586318 586319 586320 586321 586322 586323 586324 586325 586326 586327 586328 586329 586330 586331 586332 586333 586334 586335 586336 586337 586338 586339 586340 586341 586342 586343 586344 586345 586346 586347 586348 586349 586350 586351 586352 586353 586354 586355 586356 586357 586358 586359 586360 586361 586362 586363 586364 586365 586366 586367 586368 586369 586370 586371 586372 586373 586374 586375 586376 586377 586378 586379 586380 586381 586382 586383 586384 586385 586386 586387 586388 586389 586390 586391 586392 586393 586394 586395 586396 586397 586398 586399 586400 586401 586402 586403 586404 586405 586406 586407 586408 586409 586410 586411 586412 586413 586414 586415 586416 586417 586418 586419 586420 586421 586422 586423 586424 586425 586426 586427 586428 586429 586430 586431 586432 586433 586434 586435 586436 586437 586438 586439 586440 586441 586442 586443 586444 586445 586446 586447 586448 586449 586450 586451 586452 586453 586454 586455 586456 586457 586458 586459 586460 586461 586462 586463 586464 586465 586466 586467 586468 586469 586470 586471 586472 586473 586474 586475 586476 586477 586478 586479 586480 586481 586482 586483 586484 586485 586486 586487 586488 586489 586490 586491 586492 586493 586494 586495 586496 586497 586498 586499 586500 586501 586502 586503 586504 586505 586506 586507 586508 586509 586510 586511 586512 586513 586514 586515 586516 586517 586518 586519 586520 586521 586522 586523 586524 586525 586526 586527 586528 586529 586530 586531 586532 586533 586534 586535 586536 586537 586538 586539 586540 586541 586542 586543 586544 586545 586546 586547 586548 586549 586550 586551 586552 586553 586554 586555 586556 586557 586558 586559 586560 586561 586562 586563 586564 586565 586566 586567 586568 586569 586570 586571 586572 586573 586574 586575 586576 586577 586578 586579 586580 586581 586582 586583 586584 586585 586586 586587 586588 586589 586590 586591 586592 586593 586594 586595 586596 586597 586598 586599 586600 586601 586602 586603 586604 586605 586606 586607 586608 586609 586610 586611 586612 586613 586614 586615 586616 586617 586618 586619 586620 586621 586622 586623 586624 586625 586626 586627 586628 586629 586630 586631 586632 586633 586634 586635 586636 586637 586638 586639 586640 586641 586642 586643 586644 586645 586646 586647 586648 586649 586650 586651 586652 586653 586654 586655 586656 586657 586658 586659 586660 586661 586662 586663 586664 586665 586666 586667 586668 586669 586670 586671 586672 586673 586674 586675 586676 586677 586678 586679 586680 586681 586682 586683 586684 586685 586686 586687 586688 586689 586690 586691 586692 586693 586694 586695 586696 586697 586698 586699 586700 586701 586702 586703 586704 586705 586706 586707 586708 586709 586710 586711 586712 586713 586714 586715 586716 586717 586718 586719 586720 586721 586722 586723 586724 586725 586726 586727 586728 586729 586730 586731 586732 586733 586734 586735 586736 586737 586738 586739 586740 586741 586742 586743 586744 586745 586746 586747 586748 586749 586750 586751 586752 586753 586754 586755 586756 586757 586758 586759 586760 586761 586762 586763 586764 586765 586766 586767 586768 586769 586770 586771 586772 586773 586774 586775 586776 586777 586778 586779 586780 586781 586782 586783 586784 586785 586786 586787 586788 586789 586790 586791 586792 586793 586794 586795 586796 586797 586798 586799 586800 586801 586802 586803 586804 586805 586806 586807 586808 586809 586810 586811 586812 586813 586814 586815 586816 586817 586818 586819 586820 586821 586822 586823 586824 586825 586826 586827 586828 586829 586830 586831 586832 586833 586834 586835 586836 586837 586838 586839 586840 586841 586842 586843 586844 586845 586846 586847 586848 586849 586850 586851 586852 586853 586854 586855 586856 586857 586858 586859 586860 586861 586862 586863 586864 586865 586866 586867 586868 586869 586870 586871 586872 586873 586874 586875 586876 586877 586878 586879 586880 586881 586882 586883 586884 586885 586886 586887 586888 586889 586890 586891 586892 586893 586894 586895 586896 586897 586898 586899 586900 586901 586902 586903 586904 586905 586906 586907 586908 586909 586910 586911 586912 586913 586914 586915 586916 586917 586918 586919 586920 586921 586922 586923 586924 586925 586926 586927 586928 586929 586930 586931 586932 586933 586934 586935 586936 586937 586938 586939 586940 586941 586942 586943 586944 586945 586946 586947 586948 586949 586950 586951 586952 586953 586954 586955 586956 586957 586958 586959 586960 586961 586962 586963 586964 586965 586966 586967 586968 586969 586970 586971 586972 586973 586974 586975 586976 586977 586978 586979 586980 586981 586982 586983 586984 586985 586986 586987 586988 586989 586990 586991 586992 586993 586994 586995 586996 586997 586998 586999 5861000 5861010 5861020 5861030 5861040 5861050 5861060 5861070 5861080 5861090 5861100 5861110 5861120 5861130 5861140 5861150 5861160 5861170 5861180 5861190 5861200 5861210 5861220 5861230 5861240 5861250 5861260 5861270 5861280 5861290 5861300 5861310 5861320 5861330 5861340 5861350 5861360 5861370 5861380 5861390 5861400 5861410 5861420



in which  $R -$  and  $n$  are defined as above;  
or



(which is 2,2,4-trimethyl-1,3-pentanediol isobutyrate) or a combination of one or more of the above compounds with a supplemental amount of one or more other permanent high-boiling coupler solvents such as dibutyl phthalate, bis (2-ethylhexyl)phthalate, etc., exemplified, for instance, in U.S. Pat. Nos. 2,322,027, 2,533,514, 2,801,171, 2,835,579 and 3,554,755.

For purposes of preparing a coating emulsion containing one or more couplers it is also optional, though convenient, to utilize one or more low boiling auxiliary solvents to aid in initially dissolving couplers. Suitable auxiliary solvents of this type are described and exemplified, for instance, in U.S. Pat. Nos. 2,801,170, 2,801,171 and 2,949,360.

The above-defined permanent coupler solvents of this invention are generally available commercially (\*) \* (ref. Eastman Chemical Product Index; No. P143B; 14th Ed. (1972); pg. 3) or otherwise obtainable by recognized chemical steps, the (A) and (F) groups of solvents being synthesized, for instance, by refluxing an appropriate polycarboxybenzene or corresponding anhydride with an appropriate alcohol such as 2,2,4-trimethylpentanol, followed by concentration and recovery by molecular distillation.

Permanent solvents such as group (D), supra, are obtainable, for instance, by reacting pentaerithritol with methylaurate in the presence of titanium butoxide as catalyst at a molar ratio of about 1:1-4 with continuous removal of methanol-by-product.

"permanent coupler solvents" are defined as high-boiling hydrophobic coupler solvents having a boiling point of about 175 C. which are permanently retained as droplets dispersed within the silver halide emulsion layer of a color photographic element. Permanent solvents of particular interest are specifically described in the following table I-IV relating to formulae B-F supra.



or



30

TABLE I

| Coupler Solvent | R <sup>I</sup>                   | R <sup>II</sup>                  | R <sup>III</sup>              | R <sup>IV</sup>                 | R <sup>VII</sup> |
|-----------------|----------------------------------|----------------------------------|-------------------------------|---------------------------------|------------------|
| 1               | CH <sub>3</sub> -                | CH <sub>3</sub> -                | CH <sub>3</sub> -             | CH <sub>3</sub>                 | .....            |
| 2               | CH <sub>3</sub> -                | CH <sub>3</sub> -                | H                             | C <sub>4</sub> H <sub>9</sub> - | .....            |
| 3               | H                                | C <sub>2</sub> H <sub>5</sub> -  | H                             | C <sub>2</sub> H <sub>5</sub> - | .....            |
| 4               | C <sub>2</sub> H <sub>5</sub> -  | C <sub>4</sub> H <sub>9</sub> -  | H                             | H                               | .....            |
| 5               | H                                | C <sub>2</sub> H <sub>5</sub> -  | C <sub>4</sub> H <sub>9</sub> | C <sub>4</sub> H <sub>9</sub>   | .....            |
| 6               | C <sub>4</sub> H <sub>9</sub> -  | H                                | H                             | CH <sub>3</sub> -               | .....            |
| 7               | CH <sub>3</sub> -                | CH <sub>3</sub> -                | .....                         | CH <sub>3</sub> -               | .....            |
| 8               | C <sub>3</sub> H <sub>7</sub> -  | H                                | .....                         | H                               | .....            |
| 9               | CH <sub>3</sub> -                | C <sub>4</sub> H <sub>9</sub> -  | .....                         | H                               | .....            |
| 10              | CH <sub>3</sub> -                | C <sub>8</sub> H <sub>17</sub> - | .....                         | H                               | .....            |
| 11              | C <sub>2</sub> H <sub>5</sub> -  | CH <sub>3</sub> -                | .....                         | CH <sub>3</sub> -               | .....            |
| 12              | C <sub>8</sub> H <sub>17</sub> - | H                                | .....                         | H                               | .....            |



In addition, polymeric solvents such as group (C) are obtainable by heating a reactive mixture of compounds such as 2,2,4 trimethyl 1,3 pentanediol with adipic acid at a molar ratio of about 2.2 diol-to-1.0 of the acid, in the presence of a catalyst such as titanium isopropoxide with continuous removal of water, followed by the addition of about 1.1 mole of isobutyric acid.

For purposes of the present invention, it is understood that:

"supplemental amount" in reference to additional permanent coupler solvents is intended to cover about 1 percent-67 percent (by volume) of the total amount of permanent coupler solvent used in dissolving a coupler, 33 percent or less (by volume) being preferred; "low-boiling auxiliary solvent" is defined as an organic solvent of either hydrophilic or hydrophobic type which has a low-boiling point within the range of about 65 to about 160 C. and/or can be water washed from the silver halide emulsion and handled in the usual way; and

TABLE II

| Coupler Solvent | n    | R <sup>I</sup>                   | R <sup>II</sup>   | R <sup>VII</sup>                |
|-----------------|------|----------------------------------|-------------------|---------------------------------|
| 13              | 10   | CH <sub>3</sub> -                | CH <sub>3</sub> - | CH <sub>3</sub> -               |
| 14              | 50   | CH <sub>3</sub> -                | CH <sub>3</sub> - | CH <sub>3</sub> -               |
| 15              | 200  | CH <sub>3</sub> -                | CH <sub>3</sub> - | CH <sub>3</sub> -               |
| 16              | 1000 | CH <sub>3</sub> -                | CH <sub>3</sub> - | CH <sub>3</sub> -               |
| 17              | 5    | C <sub>8</sub> H <sub>17</sub> - | H                 | H                               |
| 18              | 50   | C <sub>8</sub> H <sub>17</sub> - | H                 | H                               |
| 19              | 250  | CH <sub>3</sub> -                | CH <sub>3</sub> - | CH <sub>3</sub> -               |
| 20              | 850  | CH <sub>3</sub> -                | CH <sub>3</sub> - | C <sub>2</sub> H <sub>5</sub> - |



or

TABLE II



TABLE III

| Coupler Solvent | R <sup>V</sup>                                        | R <sup>VI</sup>                         |
|-----------------|-------------------------------------------------------|-----------------------------------------|
| 21              |                                                       |                                         |
| 22              |                                                       |                                         |
| 23              |                                                       |                                         |
| 24              |                                                       |                                         |
| 25              | .....                                                 | -CO-O-CH <sub>3</sub> -                 |
| 26              | .....                                                 | -CO-O-C <sub>2</sub> H <sub>5</sub> -   |
| 27              | .....                                                 | -CO-O-C <sub>13</sub> H <sub>27</sub> - |
| 28              | .....                                                 | -CO-O-C <sub>15</sub> H <sub>31</sub> - |
| 29              | -CO-(CH <sub>2</sub> ) <sub>10</sub> -CH <sub>3</sub> |                                         |

Ballasted non-diffusible cyan dye-forming couplers suitable for use in the present invention are exemplified or suggested in U.S. Pat. Nos. 2,373,293; 2,423,730; 2,801,171; 2,895,826; 2,908,573; 3,046,129; 3,516,831; 3,311,476; 3,253,294; 3,458,315; 3,227,550; 3,476,563; 3,458,315; 3,419,390 and 3,034,892.

Useful non-diffusible magenta dye-forming couplers are exemplified or suggested, for instance, in U.S. Pat. Nos. 2,600,788; 2,801,171; 2,983,608; 2,908,573; 3,252,924; 3,311,476; 3,227,550; 3,519,429; 3,432,521; 3,419,391; 3,227,554; 3,408,194; 3,214,437; 3,152,896; 3,062,653; 3,006,759 and Belgian Patent 724,427.

Correspondingly useful non-diffusible yellow dye-forming couplers are exemplified or suggested in U.S. Pat. Nos. 2,778,658; 2,875,057; 2,908,573; 3,227,550; 3,253,924; 3,227,155; 3,408,194; 3,447,928; 3,415,652; 3,384,657; 3,369,895; 3,265,506; and 3,227,554.

For purposes of the present invention, it is also found, that DIR (Development Inhibitor Releasing) couplers can also be usefully included in the silver halide emulsion layers within the present invention. Compounds of this type are exemplified, for instance, in U.S. Pat. Nos. 3,227,554; 3,148,062 and in U.S. Ser. No. 674,090, filed on Oct. 10, 1967.

An effective amount for non-diffusible couplers of the above type can range from about 5-200 mg/ft<sup>2</sup> per emulsion layer of coated material, a concentration of 10-50 mg/ft<sup>2</sup> being generally satisfactory. Where DIR coupler is utilized in addition to 2- and/or 4-equivalent dye-forming couplers, it is found that about 5-30 mole percent of the former (i.e. DIR coupler) is adequate.

Color photographic elements within the scope of the present invention are preferably multilayered and usefully contain one or more of the following components:

A. A support layer as described, for instance, in Section X of Product Licensing Index, Vol. 92, Publication 9232 (Dec. 1971). Typical supports include cellulose acetate film, polystyrene film, polyethylene film, polypropylene film, polyethylene terephthalate film, etc.

B. Red sensitive, a green sensitive and a blue sensitive silver halide emulsion as summarized, for instance, on page 107 (Section I and III) and pages

108-9 (Section XV) of Product Licensing Index, Vol. 92, Publication 9232 (Dec. 1971). Typical suitable silver halide emulsions include silver chloride, silver bromide, silver chlorobromide, silver bromoiodide, silver chlorobromoiodide, and silver chloroiodide emulsions.

Usefully included in such emulsion layers are the usual addenda including an antistain agent such as described in U.S. Pat. No. 2,865,752.

10 C. One or more gelatin spacer layers can also be included between the light-sensitive emulsion layers and also a Carey-Lea filter layer; spacer layers of this type can optionally contain removable additives to further improve dye stability and improve color separation and

15 D. A protective gelatin overcoat layer.

The invention is further described although not limited by the following examples:

20 **EXAMPLE I**  
Fourteen light-sensitive gelatino silver halide emulsions identified as T-1 through T-14 were prepared by dissolving 76 mg of 2-[ $\alpha$ -(2,4-di-tert.-amyl-phenoxy)-butyramido]-4,6-dichloro-5-methylphenol in an equal weight of different coupler solvents (or mixtures) identified respectively as di-n-butyl phthalate (T-1-3), tributyrin (T-4), trilaurin (T-5), di-cyclohexyl phthalate (T-6), coupler solvents No. 21 (T-7), 25 (T-8), 29 (T-9), 1 (T-10), 3 (T-11), 15 (T-12), a mixture of solvent (Table V supra) No. 7 with bis (2-ethylhexyl) phthalate (66.6 percent : 33.3 percent; T-13); and a mixture of solvent No. 7 with bis(2-ethylhexyl) phthalate (33.3 percent : 66.6 percent; T-14); solution of each coupler were obtained in the usual manner in the presence of 3ml of ethyl acetate as auxiliary solvent. Each coupler solution was then mixed with 36 ml of a 6 percent aqueous gelatin solution in the presence of a surfactant, 35 the emulsified material was chill set, water washed and dried to remove auxiliary solvent and the melted dispersion blended with a light-sensitive gelatinous silver chlorobromide emulsion and applied onto a support at a concentration of 136 mg Silver/ft<sup>2</sup>, 450 mg gelatin/ft<sup>2</sup> and 78 mg coupler/ft<sup>2</sup>. Each test strip was identically exposed in an Eastman 1-B Sensitometer, developed with Developing Solution A (described below) then fixed, washed, and heat tested under wet and dry oven conditions for 14 days at 60°C./70 percent RH and for 7 days at 77°C./40 percent RH in the usual manner and loss in dye density reported in Table IV in terms of density units.

TABLE IV

| Emulsion<br>Coating No. | Coupler Solvent | $\pi_{max}$          | Dens. Loss |      |      |
|-------------------------|-----------------|----------------------|------------|------|------|
|                         |                 |                      | Dmax       | Wet  | Dry  |
| T-1-3                   | DNP*            | 670                  | 2.94       | 0.16 | **   |
|                         |                 | 665                  | 3.48       | 0.25 | 0.74 |
|                         |                 | 671                  | 2.91       | 0.19 | 0.78 |
| T-4                     | TB*             | 671                  | 2.34       | 0.08 | 0.46 |
| T-5                     | TL*             | 657                  | 2.78       | 0.09 | 0.49 |
| T-6                     | DCP*            | 667                  | 2.50       | 0.10 | **   |
| T-7                     | No. 21          | 667                  | 1.91       | 0.06 | 0.30 |
| T-8                     | No. 26          | 664                  | 2.82       | 0.06 | 0.35 |
| T-9                     | No. 29          | 658                  | 2.86       | 0.08 | 0.39 |
| T-10                    | No. 1           | 662                  | 2.96       | 0.10 | 0.31 |
| T-11                    | No. 3           | 661                  | 2.76       | 0.08 | 0.34 |
| T-12                    | No. 15          | 665                  | 2.68       | 0.10 | **   |
| T-13                    | No. 7+BEP*      | 664<br>(66.6%:33.3%) | 2.87       | 0.06 | **   |
| T-14                    | No. 7+BEP*      | 665<br>(33.3%:66.6%) | 2.87       | 0.09 | **   |

\* DNP — Di-n-butyl phthalate

TB — tributyrin

TL — trilaurin

DCP — di-cyclohexyl phthalate

BEP — bis(2-ethylhexyl) phthalate

\*\* not available

## Developing Solution A

1.0 grams surfactant  
 4.0 grams Sodium sulfite  
 3.0 grams 4-amino-N,N-diethylaniline  
 20.0 grams Sodium carbonate  
 1.72 grams NaBr  
 Water to 1.0 liter  
 pH = 10.7

### EXAMPLE II

Four test emulsions identified as T-15, T-16, T-17 and T-18 were prepared and tested as in Example I except that the incorporated couplers were the yellow dye-forming couplers (A)  $\alpha$ -pivalyl- $\alpha$ -(4-carboxyphenoxy)-2-chloro-5-[ $\gamma$ -(2,4-di-tert- $\alpha$ -amylphenoxy butyramido]-acetanilide (ref. U.S. Pat. No. 3,408,194); and (B)  $\alpha$ -pivalyl- $\alpha$ -[4-(4-benzyloxy-phenylsulfonyl) phenoxy]-2-chloro-5-[ $\gamma$ -(2,4-di-tert- $\alpha$ -amylphenoxy) butyramido]-acetanilide (ref. U.S. Pat. No. 3,408,194). The coated test films were then exposed, developed and tested identically with Example 1 and the results recorded in Table V.

TABLE V

| Emulsion<br>coating<br>number | Cou-<br>pler | Coupler<br>solvent | Dens. loss |                   |     |     |
|-------------------------------|--------------|--------------------|------------|-------------------|-----|-----|
|                               |              |                    | Max.       | D <sub>max.</sub> | Wet | Dry |
| T-15.....                     | (A)          | DNP *              | 443        | 2.75              | .17 | .12 |
| T-16.....                     | (A)          | #7 (Table I)       | 444        | 2.40              | .14 | .05 |
| T-17.....                     | (B)          | DNP *              | 449        | 2.90              | .26 | .27 |
| T-18.....                     | (B)          | #7                 | 446        | 2.34              | .08 | .10 |

The invention has been described in detail with particular reference to preferred embodiments thereof, but it will be understood that variations and modifications can be effected within the spirit and scope of the invention.

I claim:

1. In a method for forming heat stable color photographic records obtained by exposing and developing a color photographic element containing one or more light sensitive silver halide emulsion layers having at least one photographic coupler,

the improvement comprising utilizing as permanent coupler solvent a solvent system comprising at least one compound of the formulae



wherein

$R^{I-IV}$  and  $R^{VII}$  are individually defined at each occurrence as a hydrogen atom or a lower alkyl group;  $R^V$  is defined as an arylcarbonyl group or an alkylcarbonyl group;  $R^{VI}$  is defined as an alkoxy carbonyl group having up to 15 carbon atoms and  $n$  is an integer of 1-1000.

2. A method of claim 1 wherein the solvent system  
10 additionally contains a supplemental amount of a  
phthalic acid alkyl ester.

3. In a method for forming heat stable color photographic records obtained by exposing and developing a color photographic element containing one or more light  
15 sensitive silver halide emulsion layers having at least one photographic coupler,  
the improvement comprising utilizing as permanent  
20 coupler solvent at least one compound of the formulae



or



40 wherein

$R^{I-IV}$  are individually defined at each occurrence as a hydrogen atom, or an alkyl group of one to eight carbon atoms; and

$R'$  is a phenyl carbonyl group or an alkyl carbonyl group of two to 13 carbon atoms.

4. In a method for forming heat stable color photographic records obtained by exposing and developing a color photographic element containing one or more light sensitive silver halide emulsion layers having at 50 least one photographic coupler,

50 least one photographic coupler,  
the improvement comprising utilizing as permanent  
coupler solvent at least one compound of the for-  
mulae





wherein

$R'$ - $R''$  and  $R^{VII}$  are individually defined at each occurrence as a hydrogen atom or an alkyl group of one to eight carbon atoms; and  $n$  is an integer of 1-1000.

5. In a method for forming heat stable color photographic records obtained by exposing and developing a color photographic element containing one or more light sensitive silver halide emulsion layers having at least one photographic coupler

the improvement comprising utilizing as permanent coupler solvent at least one compound of the formula



wherein

$R^{VI}$  is defined as an alkoxy carbonyl group of two to 15 carbon atoms.

6. A method of claim 1 wherein the permanent coupler solvent is a member selected from the group consisting of pentaerythritol tetrabenzoate; 1,2,2,3-tetracarbethoxy propane; pentaerythritol tetralaurate; tris (2,2,4-trimethylpentyl) trimellitate; 1,2,4-benzenetricarboxylic acid, tris (2-ethylhexyl)ester; 2,2,4-trimethyl-1,3-pentanediol isobutyrate, and a 2,2,4-trimethylpentanediol-1,3-adipic acid polyester terminated with isobutyric acid.

7. A method of claim 1 wherein the solvent system contains 1-isopropyl-2,2-dimethyltrimethylene-1,3-diisobutyrate in a ratio of about 1 part by weight solvent-to-1 part by weight coupler. 40

8. A light sensitive photographic silver halide emulsion having dispersed therein finely divided particles containing at least one color photographic coupler compound in a solvent system comprising at least one compound of the formulae



wherein

$R^{I-IV}$  and  $R^{VII}$  are individually defined at each occurrence as a hydrogen atom or a lower alkyl group;  $R^V$  is defined as an arylcarbonyl group or an alkylcarbonyl group;

$R^VI$  is defined as an alkoxy carbonyl group having up to 15 carbon atoms and  $n$  is an integer of 1-1000.

9. A light sensitive photographic silver halide emulsion of claim 8 wherein the solvent system additionally contains a supplemental amount of a phthalic acid alkyl ester.

10. A light sensitive photographic silver halide emulsion of claim 8 wherein the color photographic coupler is a phenolic or  $\alpha$ -naphtholic cyan dye-forming coupler.

25 11. A light sensitive photographic silver halide emulsion of claim 8 wherein the color photographic coupler is an open chain ketomethylene yellow dye-forming coupler.

12. A light sensitive photographic silver halide emulsion of claim 8 wherein the color photographic coupler is a 5-pyrazolone magenta dye-forming coupler.

30 13. A light sensitive photographic silver halide emulsion having dispersed therein finely divided particles having at least one color photographic coupler and a permanent coupler solvent of the formulae



50 wherein

$R^I$ – $R^{IV}$  are individually defined at each occurrence as a hydrogen atom or an alkyl group of one to eight carbon atoms; and

55  $R'$  is a phenyl carbonyl group or an alkyl carbonyl group of two to 13 carbon atoms.

14. A light sensitive photographic silver halide emulsion having dispersed therein finely divided particles

containing at least one color photographic coupler compound and a permanent coupler solvent of the formulae



wherein

$R'$ – $R''$  and  $R'''$  are individually defined at each occurrence as a hydrogen atom or an alkyl group of one to eight carbon atoms; and  $n$  is an integer of 1–1000.

15. A light sensitive photographic silver halide emulsion having dispersed therein finely divided particles containing at least one photographic coupler and a permanent coupler solvent of the formula



$R^{VI}$  is defined as an alkoxy carbonyl group of two to 15 carbon atoms.

16. A light sensitive photographic silver halide emulsion of claim 8 having dispersed therein finely divided particles containing at least one coupler compound and a permanent coupler solvent selected from the group consisting of pentaerythritol tetrabenzoate; 1,2,2,3-tetracarbethoxy propane; pentaerythritol tetralaurate; tris (2,2,4-trimethylpentyl)trimellitate; 1,2,4-benzene-tricarboxylic acid, tris (2-ethylhexyl) ester; 2,2,4-trimethyl-1,3-pentanediol isobutyrate, and a 2,2,4-trimethylpentanediol-1,3-adipic acid polyester terminated with isobutyric acid.

17. A light sensitive photographic silver halide emulsion of claim 8 wherein the solvent system contains 1-isopropyl-2,2-dimethyltrimethylene-1,3-diisobutyrate in a ratio of about 1 part by weight solvent-to-1 part by weight coupler.

**18.** A light-sensitive photographic silver halide emulsion of claim 8 wherein the solvent system contains pentaerythritol tetrabenoate in a ratio of about 1 part by weight solvent-to-1 part by weight couplers.

19. A color photographic element comprising a support and at least one light-sensitive photographic silver halide emulsion layer applied thereto, said emulsion layer having dispersed therein finely divided particles containing a coupler compound in a solvent system comprising at least one compound of the formulae



12

wherein

25  $R^{I-IV}$  and  $R^{VII}$  are individually defined at each occurrence as a hydrogen atom or a lower alkyl group;  $R^V$  is defined as an arylcarbonyl group or an alkylcarbonyl group;  $R^{VI}$  is defined as an alkoxy carbonyl group having up to 15 carbon atoms and  $n$  is an integer of 1-1000.

30 20. A color photographic element of claim 19  
wherein the solvent system additionally contains a sup-  
plemental amount of a phthalic acid alkyl ester.

21. A color photographic element of claim 19 wherein the coupler compound is a phenolic- or  $\alpha$ -naphtholic-cyan dye-forming coupler.

22. A color photographic element of claim 19 wherein the coupler compound is an open chain keto-methylene yellow dye-forming coupler.

23. A color photographic element of claim 19  
40 wherein the coupler compound is a 5-pyrazolone magenta dye-forming coupler.

**24. A color photographic element comprising a sup-**

port and at least one light sensitive photographic silver halide emulsion layer applied thereto, said emulsion layer having dispersed therein finely divided particles containing a coupler compound in a solvent system comprising at least one compound of the formulae



65 wherein

$R^I$ – $R^{IV}$  are individually defined at each occurrence as a hydrogen atom or an alkyl group of one to eight carbon atoms; and  $R^V$  is a phenyl carbonyl group.

or an alkyl carbonyl group of two to 13 carbon atoms.

25. A color photographic element comprising a support and at least one light sensitive photographic silver halide emulsion layer applied thereto, said emulsion layer having dispersed therein finely divided particles containing a coupler compound in a solvent system comprising at least one compound of the formulae



wherein

$\text{R}^{\text{I}}-\text{R}^{\text{II}}$  and  $\text{R}^{\text{VII}}$  are individually defined at each occurrence as a hydrogen atom or an alkyl group of one to eight carbon atoms; and

$n$  is an integer of 1-1000.

26. A color photographic element comprising a support and at least one light sensitive photographic silver halide emulsion layer applied thereto, said emulsion layer having dispersed therein finely divided particles containing a coupler compound in a solvent system comprising at least one compound of the formula



$\text{R}^{\text{VI}}$  is defined as an alkoxy carbonyl group of two to 15 carbon atoms.

27. A color photographic element comprising a support layer and at least one light sensitive photographic silver halide emulsion layer applied thereto, said emulsion layer having dispersed therein finely divided particles containing at least one coupler compound and a permanent coupler solvent selected from the group

consisting of pentaerythritol tetrabenoate; 1,2,2,3-tetracarbethoxy propane; pentaerythritol tetralaurate; tris (2,2,4-trimethylpentyl)trimellitate; 1,2,4-benzenetricarboxylic acid, tris (2-ethylhexyl)ester; 2,2,4-trimethyl-1,3-pentanediol isobutyrate; and a 2,2,4-trimethylpentanediol-1,3-adipic acid polyester terminated with isobutyric acid.

28. A color photographic element of claim 18 wherein the solvent system contains 1-isopropyl-2,2-dimethyl-trimethylene-1,3-disobutyrate in a ratio of about 1 part by weight solvent-to-1 part by weight coupler.

29. A color photographic element of claim 18 wherein the solvent system contains pentaerythritol tetrabenoate in a ratio of about 1 part by weight solvent-to-1 part by weight coupler.

\* \* \* \* \*

40

45

50

55

60

65

UNITED STATES PATENT OFFICE  
CERTIFICATE OF CORRECTION

Patent No. 3,779,765 Dated December 18, 1973

Inventor(s) Fred C. McCrossen and Harland J. Osborn

It is certified that error appears in the above-identified patent and that said Letters Patent are hereby corrected as shown below:

Column 2, line 22 (Formula B) "(R)<sub>2</sub>" should read

--- (R<sup>I</sup>)<sub>2</sub> ---;

R<sup>I</sup>

Column 4, line 48 (Formula C), that part reading " -C- " "R<sup>II</sup>

R<sup>I</sup>

should read --- -C- ---.

Signed and sealed this 23rd day of April 1974.

(SEAL)

Attest:

EDWARD M. FLETCHER, JR.  
Attesting Officer

C. MARSHALL DANN  
Commissioner of Patents